

July 28, 1931.

G. E. SMITH

1,816,444

METHOD OF MAKING STEERING WHEELS

Filed Oct. 6, 1927

2 Sheets-Sheet 1

*Fig. 1.*



*Fig. 2.*



*Grant E. Smith Inventor*

*By his Attorneys*

*Emery Booth, Janney & Sharpe*

July 28, 1931.

G. E. SMITH

1,816,444

METHOD OF MAKING STEERING WHEELS

Filed Oct. 6, 1927

2 Sheets-Sheet 2



*Fig. 6.*

*Fig. 5.*



Inventor

Grant E. Smith

By his Attorneys

Emery Booth Janney & Stanley

## UNITED STATES PATENT OFFICE

GRANT E. SMITH, OF POUGHKEEPSIE, NEW YORK, ASSIGNOR TO POUVAILSMITH CORPORATION, OF POUGHKEEPSIE, NEW YORK, A CORPORATION OF NEW YORK

## METHOD OF MAKING STEERING WHEELS

Application filed October 6, 1927. Serial No. 224,334.

The present invention relates to wheels and to the manufacture thereof; the object of the invention being to provide a strong, durable and attractive wheel and to provide an economical and expeditious method of manufacturing the same. Inasmuch as the invention has been developed in connection with the manufacture of steering wheels for automobiles, such an embodiment has been selected for illustration and description herein.

The invention provides a novel wheel wherein the rim and spokes are constructed of moldable, preferably fibrous, material which will feel comfortable to the hand and which will have an attractive appearance. The invention provides also a novel method of manufacture whereby the wheel may be economically and expeditiously molded from a blank of a character such that it can be made from relatively inexpensive material and by steps readily adapted for expeditious manufacture not requiring a high degree of skill on the part of operatives.

The nature and objects of the invention will be better understood from the description of an illustrative embodiment thereof. In the accompanying drawings forming a part hereof—

Figure 1 is a sectional view showing a steering wheel in position in the molds in which it has been formed.

Figure 2 is a perspective view of the wheel removed from the molds.

Figure 3 is a sectional view showing a complete blank assembled in a mold previous to the molding and compressing operation.

Figure 4 is a fragmental plan view of the blank before molding.

Figure 5 is a cross-sectional view taken on the line 5—5 of Figure 3, and

Figure 6 is a detail view of a filler member of the hub blank.

The wheel shown for the purpose of illustration is compressed and molded to shape and size from a partially shaped blank of substantially larger size as shown in Figs. 3, 4 and 5. The complete blank shown is made up principally from paper impregnated with a suitable adhesive, preferably

paper of good quality such as kraft paper to provide considerable strength. The rim blank 7 as shown in the Figs. 4 and 5 is in the form of an annular roll wound with the axis of the roll substantially coincident with the axis of the wheel so that the blank when compressed in the mold is compressed edgewise of the paper. It is believed that by compressing the paper edgewise a better bond is formed.

Each spoke blank 8 consists of paper with a metal reinforcement 9 about which the paper is arranged. Preferably the paper is arranged in planes at right angles to the plane of the rim so that when compressed it is compressed edgewise of the paper. The rim is recessed as best shown in Fig. 3 to receive the end of the paper spoke and a central deeper recess being provided to receive the end of the reinforcement projecting beyond the paper. Obviously this particular arrangement may be varied as the requirements of manufacture may demand. At the inner end the metal reinforcement extends substantially into the hub. The hub blank may be formed in any suitable manner to provide a rigid structure for holding the inner ends of the spokes. In the arrangement shown, upper and lower annular rolls of paper 10 and 11 are placed respectively above and below the inner ends of the spokes, these rolls being of a simple annular form that can be conveniently and economically manufactured. The lateral spaces between the inner ends of the spokes may be suitably filled as, for example, by filler members such as shown at 12 in Fig. 6 or loose fibrous material may be introduced into the mold cavity to fill the space and provide the necessary material for forming the hub.

The blank sections should in each case be substantially thicker than the corresponding parts of the finished wheel and may be, for example, twice as thick so that the material of the blank is compressed to approximately one-half of its original volume. This provides a sufficient compacting of the material, and forms a hard durable product. The rim blank and the principal hub blanks are of such form and so designed that they can be

effectively and economically wound by machinery using paper which has been impregnated with a suitable adhesive. Crevices between the sections of the blank may be filled in with a fibrous compound such as disintegrated paper of the same character as the impregnated paper used in forming the sections of the blank. The exterior surfaces of the blank sections may be coated with additional material if desired or one may rely upon that impregnating the paper.

The impregnating material and the coating material which, if desired, may be the same, is preferably of such character that during the molding operation and without separate treatment it will become cured to form a permanent hard wear-resisting surface. A suitable phenolic condensation product or resinous material with a solvent such as methyl-alcohol may be used. It is convenient to make the solution of the material used for impregnating the paper of a very thin consistency and to make a solution of the material used for surface treatment of the blank, if any surface treatment in addition to the impregnation is desired, of the consistency of varnish. This solution may conveniently be applied by dipping. To provide a thick coating of the material on the exterior surface of the blank the blank sections or the complete assembled blank, if desired, may be redipped several times or a similar material in powdered form may be applied by dusting on after the first dipping operation and while this coating is still wet or tacky.

The assembled blank when dry is compressed and molded to form the finished wheel; the rim and hub sections being compressed about the ends of the spokes so as firmly to lock the same together. Preferably the compressing and molding operation is performed while the blank is maintained in heated condition and the compressed wheel is then cooled while still under pressure.

In the method selected for more specific description the blank is placed in the previously heated two-part mold 15, 16 and the mold is placed in a press between heated pressure heads 17, 18. After the blank has been arranged in the mold it is desirable to add additional adhesive, for example, in the form of dry powder, about the joints and if any large crevices exist to add also impregnated fibrous material in order to fill the same to make stronger and better joints. The amount of adhesive added to the parts will depend upon the character of the wheel desired and whether a substantial thickness of the adhesive is desired over the body of the structure.

The pressure heads of the press are then brought against the mold parts to press the same against the blank with a light pressure. The mold is allowed to absorb heat from the pressure heads and the blank to absorb heat

from the mold for a predetermined time, for example for five minutes, until the blank becomes thoroughly heated and then the extreme pressure is applied to close the mold and compress the complete blank to form the wheel as shown in Fig. 1. When the mold is closed and the blank fully compressed, it is cooled while still maintaining the pressure or a part of the pressure.

During the compressing and molding operation the paper or other fibrous material will flow to conform to the shape of the mold and the material of the several elements of the blank will flow into close interengaging and interlocking relation to form a rigid unitary structure.

The heat of the mold first softens and makes plastic the adhesive and then during the compressing operation the adhesive is cured and hardened. The adhesive material also acts as a lubricant between the mold and the blank and probably also between the different thicknesses of paper. The pressure employed may range, for example, from 500 to 5000 pounds per square inch of the blank to be compressed depending upon the amount of compression desired, the quality of the material of the blank, the size of the resultant object and other particular features characteristic of the material, finish or mold. The temperature at which the operation is performed may vary considerably. Successful results have been obtained by compressing kraft paper blanks at temperatures which approach 300° F. It is found convenient to heat the pressure heads by steam under a pressure of about 85 pounds per square inch circulating in suitable passages 20 therein. The molds may be cooled when the compressing operation is completed by circulating water in these same passages. The preliminary heating of the molds prior to the insertion of the blank may be accomplished in any suitable way.

The invention provides an exceptionally strong fabricated structure by reason of the compressing and molding which increases the density of the material and increases the coordination of the fibers. By the term "fabricated structure" is implied one built up of several parts connected with one another to form a complete structure. The operation of compressing the paper or other fibrous material and combining the phenolic condensation product or other equivalent material therewith produces a strong and durable wheel.

The foregoing description of a particular embodiment is illustrative merely and is not intended as defining the limits of the invention. The blank shown is merely illustrative, as obviously other material may be used for parts of the wheel, as may be desired, without departing from the spirit of the in-

vention, as defined in the appended claims.

Claims:

1. The method of making a wheel which includes assembling in a mold spoke blanks comprising paper arranged on edge, a hub blank comprising an annular paper roll and a rim blank comprising an annular paper roll, and compressing the whole under heat and pressure to approximately one-half its original volume and molding the same to form the wheel.

2. The method of making a wheel which includes assembling in a mold rim blanks, hub blanks and spoke blanks of moldable material, the spoke blanks including vertical laminæ of thin sheet material, and compressing and molding the whole under pressure to form an integral wheel.

In testimony whereof I have signed my name to this specification this 30th day of September, 1927.

GRANT E. SMITH.

25

30

35

40

45

50

55

60

65